

3,523,788  
AUSTENITIC STAINLESS STEEL OF IMPROVED  
STRESS CORROSION RESISTANCE

John F. Bates, Franklin Township, Westmoreland County,  
and Alexei W. Loginow, Monroeville Borough, Pa., as  
signors to United States Steel Corporation, a corpora-  
tion of Delaware

No Drawing. Continuation-in-part of application Ser. No.  
619,552, Mar. 1, 1967. This application June 2, 1967,  
Ser. No. 643,068

Int. Cl. C22c 39/14

U.S. Cl. 75—128

2 Claims

### ABSTRACT OF THE DISCLOSURE

The invention involves an austenitic stainless steel having outstanding stress-corrosion resistance and superior resistance to acid and pitting corrosion as well as high-temperature oxidation. The steel consists essentially of 0.05 to 0.15% carbon, 1.0 to 2.5% manganese, 0.02% max. phosphorus, 0.03% max. sulfur, 1.65 to 3.0% silicon, 8.0 to 19.0% nickel, 15.0 to 19.0% chromium, 0.05% max. nitrogen and 0.05% max. molybdenum with the aforementioned elements present according to a relationship expressed by a regression equation.

This application is a continuation-in-part of application Ser. No. 619,552 filed Mar. 1, 1967 now abandoned.

This invention relates to austenitic stainless steel. More particularly, the invention relates to an austenitic stainless steel composition which is resistant to stress-corrosion cracking, and possesses good resistance to pitting corrosion and acid corrosion as well as high-temperature oxidation.

Austenitic stainless steels have had widespread use as constructional materials in the nuclear and chemical industries. Unfortunately, in certain environments it has been shown that stress-corrosion cracking of these steels can occur. Adverse conditions such as exposure to chloride environments may precipitate stress-corrosion cracking. Obviously, because of the hazards associated with the failure of critical components in nuclear reactors and because of the expense involved in replacing components which fail in both the nuclear and chemical applications, it is desirable to provide an austenitic stainless steel having mechanical properties comparable with those of presently available austenitic stainless steels but which is resistant to stress-corrosion cracking to a greater degree. However, it is also important that such a steel be also re-

5 shown, however, that austenitic stainless steels in such cold worked, and therefore highly strained state, are less resistant to stress-corrosion cracking than the same steels in the annealed condition. It is similarly desirable, therefore, to provide an austenitic stainless steel that is resistant to stress-corrosion cracking in both the annealed and cold-worked conditions.

10 Although it is possible to minimize the problem of stress corrosion by the application of stress-relieving treatments and proper design and process control, these preventive measures are usually expensive and are not always reliable or practical. There is provided in accordance with the invention an austenitic stainless steel having a composition and structure which renders it resistant to stress-corrosion cracking without special preventive treatments, and possesses as good or greater resistance to pitting and acid corrosion than Type 304 stainless steel and a resistance to high-temperature oxidation comparable to Type 310 stainless steel. Steels in accordance with 15 the invention contain, in percent by weight, 0.05 to 0.15% carbon, 1.0 to 2.5% manganese, 0.02% max. phosphorus, 0.03% max. sulfur, 1.65 to 3.0% silicon, 8.0 to 19.0% nickel, 15.0 to 19.0% chromium, 0.05% max. nitrogen and 0.05% max. molybdenum, with the aforementioned elements present according to a relationship 20 expressed by a regression equation.

25 A presently preferred composition range of the new steel is 0.06 to 0.09% carbon, 1.0 to 2.0% manganese, 0.01% max. phosphorus, 0.01% max. sulfur, 1.8 to 2.2% silicon, 15.0 to 19.0% nickel, 17.0 to 19.0% chromium, 0.05% max. nitrogen and 0.02% max. molybdenum.

30 Several previous attempts have been made to provide the industry with an austenitic stainless steel that is resistant to stress-corrosion cracking by virtue of its composition. One such steel is disclosed in U.S. Pats. Nos. 3,159,479 and 3,159,480. Stress-corrosion resistance of this and the other presently available commercial steels is described in Table I which reports the composition and the results of stress-corrosion testing in both the cold 35 worked and annealed condition. As can be seen, some alloys have a higher resistance to stress-corrosion failure in the annealed condition but considerably less resistance in the cold-worked form. For comparison purposes, the composition of steels in accordance with the invention 40 are also provided in Table I; however, the stress-corrosion resistance properties are omitted here and will be discussed hereinafter. As will be seen, the stress-corrosion resistance of the balanced austenitic steel in accordance with the invention possesses outstanding resistance in the cold-worked condition as well as in the annealed state.

TABLE I

| Alloy                       | C      | Mn   | P     | S     | Si   | Cu     | Ni    | Cr    | Mo    | N      | Al     | Annealed | Time to failure, hours |  |
|-----------------------------|--------|------|-------|-------|------|--------|-------|-------|-------|--------|--------|----------|------------------------|--|
|                             |        |      |       |       |      |        |       |       |       |        |        |          | Cold worked            |  |
| AISI 304L                   | 0.029  | 1.28 | 0.019 | 0.015 | 0.35 | ND     | 9.52  | 18.6  | 0.19  | 0.040  | 0.02   | 5        | 2                      |  |
| AISI 316                    | 0.061  | 1.69 | 0.027 | 0.029 | 0.35 | ND     | 12.06 | 18.09 | 2.30  | 0.041  | ND     | 8        | 4                      |  |
| AISI 310                    | 0.063  | 1.15 | 0.024 | 0.013 | 0.32 | ND     | 20.0  | 24.5  | 0.15  | 0.038  | 0.01   | 15       | 11                     |  |
| Incoloy 800                 | 0.038  | 0.83 | 0.017 | 0.005 | 0.33 | 0.31   | 32.1  | 20.2  | 0.074 | 0.013  | 0.24   | 1,189    | 167                    |  |
| Patent 3,159,479 (Alloy 84) | 0.082  | 0.50 | 0.014 | 0.013 | 1.28 | <0.05  | 20.9  | 17.7  | 0.03  | 0.029  | 0.005  | NF 2,000 | 363                    |  |
| SCR                         | { 0.05 | 1.0  | Max.  | Max.  | 1.65 | { 8.0  | 15.0  | Max.  | Max.  | { 0.05 | { 0.05 |          |                        |  |
|                             | { 0.15 | 2.5  | 0.02  | 0.03  | 3.0  | { 19.0 | 19.0  | 0.05  | 0.05  | { 0.05 | { 0.05 |          |                        |  |
| SCR (Preferred)             | { 0.05 | 1.0  | Max.  | Max.  | 1.8  | { 15.0 | 17.0  | Max.  | Max.  | { 0.05 | { 0.05 |          |                        |  |
|                             | { 0.00 | 2.0  | 0.01  | 0.01  | 2.2  | { 19.0 | 19.0  | 0.02  | 0.05  | { 0.05 | { 0.05 |          |                        |  |

NOTE.—ND=Not determined; NF=No failure at indicated times; SCR=Stress corrosion resistant steel in accordance with the invention.

sistant to pitting corrosion, acid corrosion and high-temperature oxidation if it is to enjoy the generality of applications to which its outstanding properties render it well suited.

In many applications, austenitic stainless steels are used in cold-worked conditions. Typical of such uses are cold rolled and formed sheets, drawn cups and trays, as well as cold-formed tubing and piping. Experience has

65 To obtain resistance to stress-corrosion cracking with good hot workability, the steel in accordance with our invention must be balanced within the specified composition limits, with respect to the carbon, nitrogen, manganese, phosphorus, molybdenum, sulfur and silicon contents. It is necessary to maintain the carbon, manganese and silicon contents at a relatively high level and to 70 restrict the nitrogen, phosphorus, molybdenum and sulfur

contents to low levels. It is additionally important to maintain the manganese relatively high, e.g. 1% or more, for sulfur control to achieve good hot workability of the steel. It is also very important that the effects of crack-promoting elements (molybdenum, phosphorus, nitrogen, chromium and sulfur) be greatly overcome by the crack-retarding elements (nickel, carbon and silicon) for best performance in the annealed as well as in the cold worked condition. In addition, the effect of the total austenitizing elements, such as carbon, manganese, nickel and nitrogen, must be greater than that of the ferritizing elements, such as chromium, molybdenum and silicon, to render the steel predominantly austenitic at both ambient and hot-working temperatures. The austenitic structure is desirable for best cold forming and hot-working performance.

Balancing of the elements is accomplished by use of a regression equation which has been developed to describe the relationship of these elements necessary for improved stress-corrosion resistance in accordance with the invention. The regression equation for stress-corrosion behavior of austenitic stainless steels in the cold worked condition in accordance with the invention is as follows:

Natural logarithm of cracking time=

$$\begin{aligned}
 & 10.2 \\
 & -41 \text{ P} \\
 & -75 \text{ S} \\
 & +1.8 \text{ Si} \\
 & +0.33 \text{ Ni} \\
 & -0.60 \text{ Cr} \\
 & -13 \text{ Mo} \\
 & +23 (\text{P}-0.016) (\text{Si}-1.1) \\
 & -6.1 (\text{P}-0.016) (\text{Ni}-16) \\
 & -0.0058 (\text{Ni}-16)^2
 \end{aligned}$$

Error in prediction at the 95% probability limit =  $\pm 0.92$   
Coefficient of determination ( $R^2$ ) = 95.9%.

The aforementioned regression equation which was developed after extensive investigation relates the compositional effects to the failure times of cold-worked specimens. A logarithm transformation was made on the mean cracking times prior to analysis and the equation is expressed in terms of natural log cracking time. A positive sign associated with single element effects and interaction effects indicates a beneficial effect, and a negative sign indicates a detrimental effect. The interaction effects included in the regression equations indicate that the effect on the cracking time of one chemical element differs at different levels of another element. Those knowledgeable in the art will appreciate that there is usually a wide spread in stress-corrosion data. To indicate the high level of reliability, also included above, are a measure of the error in predicting the natural log cracking time at the 95% probability limit and a measure ( $R^2$ ) of the percent of total variation in the natural logarithm of the cracking time explained by the composition effects.

We have found that the desirable combination of stress-corrosion resistance and hot workability can be achieved if the composition is critically controlled within the relationship described by the aforementioned regression equation with each element present within the ranges previously given. Moreover, we have discovered that manganese need not be, as has been previously believed, detrimental to stress corrosion resistance, and it is possible to include the relatively high manganese level necessary for improved hot workability. Thus, with silicon within the range of 1.65 to 3.0%, manganese contents within the range of 1.0 to 2.5% may be maintained without sacrificing resistance to stress-corrosion cracking and will result in outstanding hot workability for these types of steels.

We have also discovered that it is necessary to restrict molybdenum to relatively low levels on the order of 0.05% max. to provide the desired resistance to stress-

corrosion cracking. In addition, for good resistance to corrosion and high-temperature oxidation, the steel should contain sufficient chromium (up to about 19%) although lower contents of chromium (about 15%) would impart improved stress-corrosion performance. Nickel is added to the steel to ensure an austenitic structure, high ductility, good cold-working properties and resistance to stress-corrosion cracking. Although greater amounts of nickel, i.e. 20% or more, are beneficial to obtain increased resistance to stress-corrosion cracking, we have found that the detrimental effects of phosphorus are more pronounced at increasing nickel levels and, of course, hot workability suffers. The nickel content of the balanced steel composition in accordance with the invention is maintained at a level such that the steel still has good hot workability. The carbon content is controlled closely at a relatively high level to provide austenite stabilization and resistance to stress-corrosion cracking. The nitrogen content of the steel is kept at a low level. For best resistance to stress-corrosion cracking, the nitrogen content is preferably lower than 0.05%. The phosphorus content is kept below 0.01% for resistance to stress-corrosion cracking of the cold-worked steel and the silicon content is kept as high as is consistent with good hot-working characteristics. Sulfur is kept low for hot workability and for resistance to stress-corrosion cracking. Other elements, such as copper and aluminum, when contained in the new steel, are present in the small amounts normally present in 18% chromium, 8% nickel (AISI Type 304) austenitic stainless steels.

The following examples will aid in understanding the invention.

For the examples, heats were melted in an induction furnace and hot rolled to  $\frac{1}{2}$ -inch thick plate. Specimen blanks ( $\frac{1}{2} \times \frac{1}{2} \times 3\frac{1}{2}$ -inches) were cut with the long dimension parallel to the rolling direction. The blanks were solution annealed and water quenched. Tension specimens, 0.252-inch in diameter, were machined from the blanks. Some of the specimens were tested in the annealed condition by loading to 75% of the yield strength. Other specimens were elongated 30% in a tensile machine and tested in a cold-worked condition by loading to 75% of the new yield strength. A standard hot salt test was used in which the specimens were totally immersed in a boiling 42% magnesium chloride solution.

Usually three specimens were tested in the annealed and three in the cold-worked condition for each heat. Cold-worked specimens were removed after a minimum of 2000 hours if they had not failed; annealed specimens were removed after times varying from 2000 to 4500 hours if there had been no failure. The mean times to failure were used to evaluate the materials. Where some specimens from a given heat failed and others did not fail, there is no simple mean that will satisfactorily describe such behavior. Consequently, the value used was arbitrarily chosen to be the mean of the times to failure and the "no-failure" times; such values are indicated as erratic (E) in the tables to recognize the inadequacy of the numerical value. Unlike other alloys, austenitic steels in accordance with the invention may provide a time-to-failure in the cold-worked condition of as much as 450 hours or more when tested as described above.

The compositions and the stress-corrosion behavior of a series of known steels, as discussed previously, are given in Table I above. One composition is a melted heat within the range of the aforementioned U.S. Pat. No. 3,159,479. It is noted that although steel of typical compositions within the aforementioned patent have good resistance to stress-corrosion cracking in the annealed condition, resistance in the cold-worked condition is limited. Moreover, as will be hereinafter pointed out, steel in accordance with the invention possesses good resistance to acid and pitting corrosion as well as to high-temperature oxidation. Thus, a superior characteristic of steels

in accordance with the invention is the unique combination of outstanding properties with respect to (1) stress-corrosion resistance, (2) pitting-corrosion resistance, (3) acid-corrosion resistance, and (4) high-temperature oxi-

phorus and molybdenum had not been included. However, the improvement obtained by increasing the nickel content to within the range specified for our steels is clearly indicated.

TABLE II.—EFFECT OF NICKEL

| Alloy | Composition, percent |      |       |       |      |       |      |      |       |       |       | Time to failure, hours |             |
|-------|----------------------|------|-------|-------|------|-------|------|------|-------|-------|-------|------------------------|-------------|
|       | C                    | Mn   | P     | S     | Si   | Cu    | Ni   | Cr   | Mo    | N     | Al    | Annealed               | Cold worked |
| 5     | 0.019                | 1.50 | 0.027 | 0.015 | 0.53 | <0.01 | 7.87 | 17.6 | <0.01 | 0.035 | 0.004 | 46                     | 3           |
| 16    | 0.010                | 1.43 | 0.021 | 0.018 | 0.48 | <0.01 | 13.0 | 17.1 | <0.01 | 0.047 | 0.10  | 69                     | 9           |
| 11    | 0.017                | 1.50 | 0.023 | 0.021 | 0.49 | <0.01 | 17.8 | 17.6 | <0.01 | 0.036 | 0.015 | 76                     | 38          |
| 14    | 0.057                | 1.51 | 0.024 | 0.017 | 0.50 | <0.01 | 7.85 | 17.6 | <0.01 | 0.043 | 0.10  | 4                      | 2           |
| 18    | 0.065                | 1.60 | 0.021 | 0.019 | 0.52 | <0.01 | 17.7 | 17.1 | <0.01 | 0.037 | 0.11  | 378                    | 50          |

NOTE.—NF=No failure at indicated times.

#### dation resistance.

The criticality of the composition may be seen by examples wherein the effects of the individual elements is demonstrated. Some elements (phosphorus, sulfur, silicon, chromium and molybdenum) were found to affect the stress-corrosion resistance of the cold-worked material only, some (carbon and nitrogen) the resistance of annealed material only, and one (nickel) the resistance of both. The present steel provides resistance to stress-corrosion cracking in both annealed and cold-worked conditions.

It is generally known that high nickel content in-

Carbon is a beneficial element in stress-corrosion resistance as indicated by the data shown in Table III. As can be seen by comparing the annealed condition properties, maintaining carbon over about 0.05% materially improves stress-corrosion resistance. It is also noted that the high carbon content is desirable for the beneficial effect of low nitrogen to become operative (carbon-nitrogen interaction). In comparison Groups A, B, C and D, increased carbon improved the stress-corrosion resistance in the annealed condition. In three of the five comparison groups, Groups B, D and E, carbon is shown to be distinctly beneficial for cold worked material.

TABLE III.—EFFECT OF CARBON

| Group | Alloy | Composition, percent |      |       |       |      |       |      |      |       |       |       | Time to failure, hours |             |
|-------|-------|----------------------|------|-------|-------|------|-------|------|------|-------|-------|-------|------------------------|-------------|
|       |       | C                    | Mn   | P     | S     | Si   | Cu    | Ni   | Cr   | Mo    | N     | Al    | Annealed               | Cold worked |
| A     | 9     | 0.034                | 1.53 | 0.025 | 0.017 | 0.53 | <0.01 | 17.8 | 17.8 | <0.01 | 0.006 | 0.004 | 220                    | 38          |
|       | 10    | 0.073                | 1.55 | 0.029 | 0.015 | 0.50 | <0.01 | 17.9 | 17.8 | <0.01 | 0.005 | 0.010 | NF 4,500               | 48          |
| B     | 1     | 0.010                | 2.39 | 0.005 | 0.011 | 0.19 | <0.01 | 18.1 | 16.4 | <0.01 | 0.007 | 0.007 | 627                    | 138         |
|       | 2     | 0.07                 | 2.53 | 0.007 | 0.011 | 0.24 | <0.01 | 17.9 | 17.3 | <0.01 | 0.010 | 0.012 | NF 3,300               | 520         |
| C     | 3     | 0.044                | 1.51 | 0.025 | 0.017 | 0.49 | <0.01 | 7.9  | 17.6 | <0.01 | 0.005 | 0.011 | 921                    | 4           |
|       | 4     | 0.075                | 1.50 | 0.028 | 0.012 | 0.50 | <0.01 | 8.0  | 17.7 | <0.01 | 0.006 | 0.008 | NF 4,500               | 2           |
| D     | 90    | 0.021                | 1.53 | 0.008 | 0.014 | 1.96 | 0.11  | 18.2 | 17.8 | 0.028 | 0.033 | 0.011 | 974                    | 223         |
|       | 75    | 0.074                | 1.52 | 0.007 | 0.013 | 1.99 | 0.10  | 18.1 | 18.5 | 0.030 | 0.035 | 0.010 | NF 2,000               | E 1,649     |
| E     | 21    | 0.053                | 1.44 | 0.010 | 0.016 | 0.28 | 0.01  | 17.2 | 17.9 | 0.015 | 0.009 | 0.021 | NF 4,600               | 50          |
|       | 22    | 0.075                | 1.44 | 0.008 | 0.019 | 0.34 | <0.01 | 18.3 | 17.6 | 0.015 | 0.011 | 0.008 | NF 4,600               | 96          |

NOTE.—NF=No failure at indicated times; E=Erratic behavior.

creases resistance of austenitic stainless steels to stress-corrosion cracking in hot chloride solutions. However, very high nickel contents, i.e. 20% or greater, are not desirable because of a detrimental nickel-phosphorus interaction which is hereinafter discussed with the effects of phosphorus and because of the detrimental effect on hot workability.

The effect of nickel is shown in Table II which is divided into two groups of data, and each group is a comparison series with increasing nickel content. It will be noted that for both cold worked and annealed material, increasing nickel content is beneficial. The properties of these steels are all poorer than the optimum composition because the optimum contents of silicon, phos-

The effect of silicon is shown in Table IV which indicates that silicon is beneficial in the cold-worked material but has a less significant effect in the annealed material. However, with a crack-promoting element (molybdenum) at a high level, the beneficial effect of silicon in the annealed condition is clearly evident. An interaction of the beneficial silicon effect with the detrimental phosphorus effect is discussed with effects of phosphorus. It will be seen from Table IV that the first two groups at the 9% nickel level show little effect of increasing silicon from the 0.4 to the 0.9% level. However, increase of silicon to 2.0% was invariably beneficial at the 18% nickel level. The last two comparison groups show the great advantage of having silicon higher than 1.65%.

TABLE IV.—Effect of Silicon

| Alloy   | Composition, percent |      |       |       |      |       |      |      |       |       |       | Time to failure, hours |             |
|---------|----------------------|------|-------|-------|------|-------|------|------|-------|-------|-------|------------------------|-------------|
|         | C                    | Mn   | P     | S     | Si   | Cu    | Ni   | Cr   | Mo    | N     | Al    | Annealed               | Cold worked |
| 35..... | 0.094                | 1.53 | 0.003 | 0.015 | 0.45 | <0.02 | 9.05 | 18.9 | <0.01 | 0.012 | 0.012 | NF 2,000               | 2           |
| 36..... | 0.096                | 1.56 | 0.003 | 0.015 | 0.89 | <0.02 | 9.05 | 18.7 | <0.01 | 0.014 | 0.015 | NF 2,000               | 2           |
| 37..... | 0.084                | 1.55 | 0.031 | 0.016 | 0.41 | <0.05 | 8.90 | 17.0 | <0.01 | 0.010 | 0.017 | E 1,371                | 2           |
| 39..... | 0.091                | 1.52 | 0.030 | 0.016 | 0.86 | <0.05 | 8.88 | 16.9 | <0.01 | 0.011 | 0.017 | NF 2,000               | 6           |
| 84..... | 0.082                | 0.50 | 0.014 | 0.013 | 1.28 | <0.05 | 20.9 | 17.7 | 0.03  | 0.029 | 0.005 | NF 2,000               | 363         |
| 79..... | 0.081                | 1.45 | 0.014 | 0.013 | 2.00 | 0.10  | 17.8 | 17.8 | 0.034 | 0.036 | 0.009 | NF 2,000               | 674         |
| 26..... | 0.095                | 1.51 | 0.025 | 0.017 | 0.40 | <0.05 | 17.7 | 18.0 | <0.01 | 0.010 | 0.016 | NF 2,000               | 81          |
| 29..... | 0.095                | 1.52 | 0.026 | 0.017 | 1.98 | <0.05 | 18.1 | 18.0 | <0.01 | 0.009 | 0.010 | NF 2,000               | 786         |
| 43..... | 0.076                | 1.56 | 0.010 | 0.017 | 0.47 | 0.10  | 17.6 | 17.7 | 0.22  | 0.058 | 0.010 | 62                     | 25          |
| 44..... | 0.081                | 1.56 | 0.014 | 0.012 | 1.77 | 0.10  | 18.1 | 17.9 | 0.22  | 0.057 | 0.019 | 1,033                  | 68          |
| 88..... | 0.078                | 1.47 | 0.010 | 0.016 | 0.90 | 0.10  | 17.6 | 17.6 | 0.030 | 0.042 | 0.003 | NF 2,000               | 100         |
| 89..... | 0.077                | 1.47 | 0.010 | 0.015 | 1.44 | 0.10  | 17.5 | 17.8 | 0.030 | 0.038 | 0.003 | -----                  | 209         |
| 83..... | 0.077                | 1.51 | 0.009 | 0.014 | 2.05 | 0.10  | 17.8 | 18.0 | 0.026 | 0.034 | 0.005 | NF 2,000               | 1,012       |

NOTE.—NF=No failure at indicated times; E=Erratic behavior.

As the single element variation data in Table V indicates, molybdenum is markedly detrimental in the cold-worked condition.

The normal residual molybdenum content in commercial austenitic stainless steels made from a scrap charge usually is in the range 0.1 to 0.5%. In the examples, this is represented by 0.2% molybdenum. It can be seen from the three comparison groups in Table V that molybdenum at the normal residual levels is very detrimental. The first group also indicates that lowering the molybdenum to as low a level as is presently technologically possible, even below 0.015%, will result in further increases in stress-corrosion resistance.

such that the detrimental effect of phosphorus becomes less pronounced as the silicon content increases. A phosphorus-nickel interaction also occurs with the result that the detrimental effect of phosphorus becomes more pronounced as the nickel content increases. This interaction is of very great importance in itself and in context with other discoveries described herein. Moreover, these interactions very closely point up the necessity of critically controlling the composition. Thus, the content of each element must be counterbalanced in accordance with the regression equation by other elements for an optimum combination of properties.

The single element comparisons of various phosphorus contents shown in Table VI are divided into seven com-

TABLE V.—Effect of Molybdenum

| Alloy   | Composition, percent |      |       |       |      |       |      |      |       |       |       | Time to failure, hours |             |
|---------|----------------------|------|-------|-------|------|-------|------|------|-------|-------|-------|------------------------|-------------|
|         | C                    | Mn   | P     | S     | Si   | Cu    | Ni   | Cr   | Mo    | N     | Al    | Annealed               | Cold worked |
| 30..... | 0.088                | 1.52 | 0.010 | 0.016 | 0.42 | <0.05 | 17.9 | 18.4 | <0.01 | 0.009 | 0.012 | NF 2,100               | E 976       |
| 22..... | 0.075                | 1.44 | 0.008 | 0.019 | 0.34 | <0.01 | 18.4 | 17.6 | 0.015 | 0.011 | 0.008 | NF 4,600               | 96          |
| 73..... | 0.074                | 1.89 | 0.008 | 0.026 | 1.94 | 0.10  | 17.8 | 17.9 | 0.028 | 0.043 | 0.008 | NF 2,000               | 408         |
| 45..... | 0.075                | 1.60 | 0.006 | 0.016 | 1.89 | 0.09  | 17.7 | 17.5 | 0.22  | 0.043 | 0.007 | NF 2,200               | 67          |
| 78..... | 0.075                | 1.45 | 0.008 | 0.013 | 2.00 | 0.10  | 17.8 | 17.7 | 0.033 | 0.031 | 0.009 | NF 2,000               | 814         |
| 82..... | 0.079                | 1.45 | 0.010 | 0.012 | 1.98 | 0.10  | 17.9 | 17.7 | 0.072 | 0.032 | 0.007 | NF 2,000               | 368         |
| 59..... | 0.072                | 1.50 | 0.010 | 0.012 | 1.99 | 0.11  | 18.0 | 17.6 | 0.21  | 0.027 | 0.011 | NF 2,000               | 106         |

NOTE.—NF=No failure at indicated times; E=Erratic behavior.

The effects of phosphorus are shown in Table VI. These examples demonstrate that phosphorus is quite detrimental in the cold-worked material, but is somewhat detrimental in the annealed state when the molybdenum content is relatively high. A phosphorus-silicon interaction occurs

parison groups. Especially noteworthy is the first comparison group of four heats which were made as a split heat, varying only phosphorus. Without exception, each group shows phosphorus to be detrimental in the cold-worked state.

TABLE VI.—Effect of Phosphorus

| Alloy   | Composition, percent |      |       |       |      |       |      |      |       |       | Time to failure, hours |          |             |
|---------|----------------------|------|-------|-------|------|-------|------|------|-------|-------|------------------------|----------|-------------|
|         | C                    | Mn   | P     | S     | Si   | Cu    | Ni   | Cr   | Mo    | N     | Al                     | Annealed | Cold worked |
| 58..... | 0.052                | 1.48 | 0.006 | 0.011 | 2.02 | 0.11  | 18.0 | 17.9 | 0.21  | 0.026 | 0.009                  | NF 2,000 | 119         |
| 59..... | 0.072                | 1.50 | 0.010 | 0.012 | 1.99 | 0.11  | 18.0 | 17.6 | 0.21  | 0.027 | 0.011                  | NF 2,000 | 106         |
| 61..... | 0.058                | 1.48 | 0.020 | 0.012 | 2.00 | 0.11  | 18.0 | 17.9 | 0.22  | 0.028 | 0.012                  | 1,235    | 81          |
| 62..... | 0.087                | 1.49 | 0.022 | 0.011 | 1.98 | 0.11  | 17.9 | 17.9 | 0.21  | 0.029 | 0.009                  | 916      | 70          |
| 77..... | 0.078                | 1.46 | 0.004 | 0.014 | 1.97 | 0.10  | 17.8 | 17.7 | 0.034 | 0.030 | 0.010                  | NF 2,000 | E 1,208     |
| 78..... | 0.075                | 1.45 | 0.008 | 0.013 | 2.00 | 0.10  | 17.8 | 17.7 | 0.033 | 0.031 | 0.009                  | NF 2,000 | 814         |
| 79..... | 0.081                | 1.45 | 0.014 | 0.013 | 2.00 | 0.10  | 17.8 | 17.8 | 0.034 | 0.036 | 0.009                  | NF 2,000 | 674         |
| 80..... | 0.082                | 1.45 | 0.004 | 0.014 | 1.85 | 0.10  | 17.9 | 17.7 | 0.074 | 0.030 | 0.005                  | NF 2,000 | 428         |
| 81..... | 0.082                | 1.45 | 0.011 | 0.012 | 1.81 | 0.10  | 17.9 | 17.6 | 0.072 | 0.030 | 0.008                  | NF 2,000 | 353         |
| 82..... | 0.079                | 1.45 | 0.010 | 0.012 | 1.98 | 0.10  | 17.9 | 17.7 | 0.072 | 0.032 | 0.007                  | NF 2,000 | 368         |
| 30..... | 0.088                | 1.52 | 0.010 | 0.016 | 0.42 | <0.05 | 17.9 | 18.4 | <0.01 | 0.009 | 0.012                  | NF 2,000 | E 976       |
| 26..... | 0.095                | 1.51 | 0.025 | 0.017 | 0.40 | <0.05 | 17.7 | 18.0 | <0.01 | 0.010 | 0.016                  | NF 2,000 | 81          |
| 23..... | 0.083                | 1.63 | 0.009 | 0.008 | 1.94 | 0.030 | 18.1 | 18.0 | <0.01 | 0.009 | 0.026                  | NF 2,100 | NF 2,100    |
| 29..... | 0.095                | 1.52 | 0.026 | 0.017 | 1.98 | <0.05 | 18.1 | 18.0 | <0.01 | 0.009 | 0.010                  | NF 2,000 | 786         |
| 25..... | 0.067                | 1.50 | 0.007 | 0.014 | 1.92 | <0.01 | 17.5 | 17.3 | <0.01 | 0.021 | 0.005                  | NF 2,000 | NF 2,000    |
| 48..... | 0.082                | 1.45 | 0.030 | 0.013 | 1.96 | <0.01 | 17.4 | 17.5 | <0.01 | 0.022 | 0.011                  | -----    | 841         |
| 2.....  | 0.07                 | 2.53 | 0.007 | 0.011 | 0.24 | <0.01 | 17.9 | 17.3 | <0.01 | 0.010 | 0.012                  | NF 3,300 | 520         |
| 10..... | 0.073                | 1.55 | 0.029 | 0.015 | 0.50 | <0.01 | 17.9 | 17.8 | <0.01 | 0.005 | 0.010                  | NF 4,500 | 48          |

NOTE.—NF=No failure at indicated time; E=Erratic behavior.

It has been found that nitrogen is detrimental in the annealed material, but that the effect for cold-worked material is too small to be significant. A carbon-nitrogen interaction for annealed steels occurs such that the beneficial effect of low nitrogen content is less pronounced at low carbon levels and the beneficial effect of carbon is less pronounced at high nitrogen levels. Technological considerations limit the lowest practical level for nitrogen and metallurgical factors, such as intergranular carbide precipitation, control the upper limit for carbon.

In Table VII the first and second comparison groups are split heats varying only in nitrogen. The stress-corrosion behavior of the steels in the first group are rather poor

because all of these heats are high in molybdenum (0.22%). The second comparison group represents additions of nitrogen above the levels normally encountered in commercial austenitic stainless steels (0.03 to 0.05% N). Both of these groups, however, indicate a detrimental effect for nitrogen in the cold-worked condition.

The fourth comparison group, with up to 0.021% nitrogen, comprises steels that did not fail in the cold-worked condition. These steels, however, contain a very low level of molybdenum, less than 0.01%. The last two comparison groups show the marked detrimental effect of nitrogen on annealed steels having low nickel and high phosphorus contents.

TABLE VII.—EFFECT OF NITROGEN

| Alloy   | Composition, percent |      |       |       |      |       |      |      |       |       | Time to failure, hours |          |             |
|---------|----------------------|------|-------|-------|------|-------|------|------|-------|-------|------------------------|----------|-------------|
|         | C                    | Mn   | P     | S     | Si   | Cu    | Ni   | Cr   | Mo    | N     | Al                     | Annealed | Cold worked |
| 49..... | 0.069                | 1.50 | 0.011 | 0.012 | 2.01 | 0.11  | 18.0 | 17.7 | 0.22  | 0.005 | 0.008                  | NF 2,000 | 129         |
| 50..... | 0.071                | 1.50 | 0.011 | 0.013 | 2.04 | 0.10  | 18.0 | 17.8 | 0.22  | 0.010 | 0.010                  | E 1,300  | 115         |
| 52..... | 0.072                | 1.50 | 0.013 | 0.014 | 2.08 | 0.11  | 18.0 | 17.7 | 0.22  | 0.015 | 0.009                  | E 1,450  | 110         |
| 54..... | 0.068                | 1.50 | 0.007 | 0.011 | 2.03 | 0.11  | 18.0 | 17.6 | 0.22  | 0.025 | 0.010                  | NF 2,000 | 96          |
| 56..... | 0.051                | 1.50 | 0.008 | 0.010 | 1.98 | 0.11  | 18.0 | 17.8 | 0.22  | 0.036 | 0.010                  | E 1,500  | 79          |
| 85..... | 0.081                | 1.48 | 0.011 | 0.016 | 2.04 | 0.10  | 19.6 | 17.7 | 0.028 | 0.052 | 0.006                  | NF 2,000 | 526         |
| 86..... | 0.084                | 1.48 | 0.010 | 0.016 | 2.02 | 0.10  | 19.6 | 17.6 | 0.026 | 0.072 | 0.006                  | NF 2,000 | 253         |
| 87..... | 0.080                | 1.48 | 0.006 | 0.017 | 2.06 | 0.10  | 19.6 | 17.7 | 0.028 | 0.105 | 0.005                  | NF 2,000 | 141         |
| 22..... | 0.075                | 1.44 | 0.008 | 0.019 | 0.34 | <0.01 | 18.4 | 17.6 | 0.015 | 0.011 | 0.008                  | NF 4,600 | 96          |
| 42..... | 0.070                | 1.49 | 0.013 | 0.024 | 0.37 | <0.02 | 18.2 | 17.7 | 0.017 | 0.030 | 0.010                  | NF 2,000 | 69          |
| 23..... | 0.083                | 1.63 | 0.009 | 0.008 | 1.94 | 0.030 | 18.1 | 18.1 | <0.01 | 0.009 | 0.026                  | NF 2,100 | NF 2,100    |
| 24..... | 0.080                | 1.46 | 0.010 | 0.013 | 1.86 | <0.01 | 17.4 | 17.8 | <0.01 | 0.015 | 0.007                  | NF 2,000 | NF 2,000    |
| 25..... | 0.087                | 1.50 | 0.007 | 0.014 | 1.92 | <0.01 | 17.5 | 17.3 | <0.01 | 0.021 | 0.005                  | NF 2,000 | NF 2,000    |
| 72..... | 0.072                | 1.62 | 0.003 | 0.016 | 1.95 | 0.10  | 17.4 | 17.5 | 0.033 | 0.019 | 0.005                  | NF 2,000 | E 1,728     |
| 71..... | 0.065                | 1.42 | 0.003 | 0.015 | 1.90 | 0.10  | 17.8 | 17.8 | 0.035 | 0.028 | 0.003                  | NF 2,000 | 823         |
| 77..... | 0.078                | 1.46 | 0.004 | 0.014 | 1.97 | 0.10  | 17.8 | 17.7 | 0.034 | 0.030 | 0.010                  | NF 2,000 | E 1,208     |
| 74..... | 0.072                | 1.54 | 0.009 | 0.015 | 1.99 | 0.10  | 18.0 | 18.1 | 0.030 | 0.017 | 0.010                  | NF 2,000 | 752         |
| 78..... | 0.075                | 1.45 | 0.008 | 0.013 | 2.00 | 0.10  | 17.8 | 17.7 | 0.033 | 0.031 | 0.009                  | NF 2,000 | 814         |
| 73..... | 0.074                | 1.89 | 0.008 | 0.026 | 1.94 | 0.10  | 17.8 | 17.9 | 0.028 | 0.043 | 0.008                  | NF 2,000 | 408         |
| 4.....  | 0.075                | 1.50 | 0.028 | 0.012 | 0.50 | <0.01 | 8.0  | 17.7 | <0.01 | 0.006 | 0.008                  | NF 4,500 | 29          |
| 14..... | 0.057                | 1.51 | 0.024 | 0.017 | 0.50 | <0.01 | 7.9  | 17.6 | <0.01 | 0.043 | 0.100                  | 4        | 72          |
| 10..... | 0.073                | 1.55 | 0.029 | 0.015 | 0.50 | <0.01 | 17.9 | 17.8 | <0.01 | 0.005 | 0.010                  | NF 4,500 | 48          |
| 18..... | 0.065                | 1.60 | 0.021 | 0.019 | 0.52 | <0.01 | 17.7 | 17.1 | <0.01 | 0.037 | 0.110                  | 378      | 50          |

NOTE.—NF=No failure at indicated times; E=Erratic behavior.

We have also observed that increasing chromium above about 19% is detrimental in cold-worked material. Thus, it is desirable to have as low chromium as possible consistent with the needed resistance to general corrosion. Sulfur in the range 0.01 to 0.02% is also detrimental for cold-worked materials and, therefore, the sulfur content should be kept as low as possible. Furthermore, a low sulfur content improves the hot-working properties of the steel. Manganese in the range 1.0 to 2.5%, aluminum in the range 0.005 to 0.03% and copper in the range 0.01 to 0.12% do not have a significant effect on stress-corrosion behavior.

A number of steels within the scope of the invention are

A test for pitting corrosion is conducted in an acidified ferric chloride solution (108 g.  $\text{FeCl}_3 \cdot 6\text{H}_2\text{O}$ , 4.5 ml. conc. HCl per liter of solution) for 4 hours at 95° F. A series of specimens of the composition of steels shown in Table IX were treated in the test solution and the weight loss of the specimens was calculated as milligrams per square decimeter per day (m.d.d.), a unit commonly used for non-uniform (pitting) corrosion testing. The results of the test are reported in Table X and as can be seen, Alloy 78, a composition in accordance with the invention, had a somewhat lower corrosion rate than Type 304 stainless steel and an appreciably lower corrosion rate than Alloy 84.

TABLE IX.—STAINLESS STEELS TESTED

| Alloy    | C     | Mn   | P     | S     | Si   | Cu    | Ni   | Cr   | Mo    | Al    | N     |
|----------|-------|------|-------|-------|------|-------|------|------|-------|-------|-------|
| 78       | 0.075 | 1.45 | 0.008 | 0.013 | 2.00 | 0.10  | 17.8 | 17.7 | 0.03  | 0.009 | 0.038 |
| 84       | 0.082 | 0.50 | 0.014 | 0.013 | 1.28 | <0.05 | 20.9 | 17.7 | 0.03  | 0.005 | 0.021 |
| Type 304 | 0.049 | 1.79 | 0.029 | 0.011 | 0.25 | 0.14  | 9.59 | 18.4 | 0.16  | ND    | 0.039 |
| Type 310 | 0.052 | 1.47 | 0.016 | 0.016 | 0.67 | ND    | 20.1 | 24.4 | 0.086 | ND    | 0.026 |

NOTE.—ND=Not determined.

summarized in Table VIII. These examples show that varying degrees of resistance to stress-corrosion cracking may be obtained within the limits imposed by our invention. However, they also show that the steels of our invention have a considerably better resistance to stress-corrosion cracking in both annealed and cold-worked conditions than currently available steels also presented in the table, and in particular, in the cold-worked condition a time-to-failure of greater than 450 hours.

TABLE VIII

| Alloy                             | Composition, percent |      |       |       |      |      |       |       |       |       | Time to failure, hours |          |             |
|-----------------------------------|----------------------|------|-------|-------|------|------|-------|-------|-------|-------|------------------------|----------|-------------|
|                                   | C                    | Mn   | P     | S     | Si   | Cu   | Ni    | Cr    | Mo    | N     | Al                     | Annealed | Cold worked |
| Stress Corrosion Resistant Steels |                      |      |       |       |      |      |       |       |       |       |                        |          |             |
| 23                                | 0.083                | 1.63 | 0.009 | 0.008 | 1.94 | 0.03 | 18.1  | 18.0  | <0.01 | 0.009 | 0.026                  | NF 2,100 | NF 2,100    |
| 24                                | 0.080                | 1.46 | 0.010 | 0.013 | 1.86 | 0.01 | 17.4  | 17.3  | <0.01 | 0.015 | 0.007                  | NF 2,000 | NF 2,000    |
| 25                                | 0.067                | 1.50 | 0.007 | 0.014 | 1.92 | 0.01 | 17.5  | 17.3  | <0.01 | 0.021 | 0.005                  | NF 2,000 | NF 2,000    |
| 72                                | 0.072                | 1.62 | 0.003 | 0.016 | 1.95 | 0.10 | 17.4  | 17.5  | 0.033 | 0.019 | 0.005                  | NF 2,000 | E 1,728     |
| 76                                | 0.080                | 1.51 | 0.007 | 0.013 | 1.92 | 0.10 | 18.4  | 18.3  | 0.031 | 0.032 | 0.010                  | NF 2,000 | E 1,486     |
| 75                                | 0.074                | 1.52 | 0.007 | 0.013 | 1.99 | 0.10 | 18.1  | 18.5  | 0.030 | 0.035 | 0.010                  | NF 2,000 | E 1,64      |
| 77                                | 0.078                | 1.46 | 0.004 | 0.014 | 1.97 | 0.10 | 17.8  | 17.7  | 0.034 | 0.030 | 0.010                  | NF 2,000 | E 1,208     |
| 83                                | 0.077                | 1.51 | 0.009 | 0.014 | 2.05 | 0.10 | 17.8  | 18.0  | 0.026 | 0.034 | 0.005                  | NF 2,000 | 1,013       |
| 71                                | 0.065                | 1.42 | 0.003 | 0.015 | 1.90 | 0.10 | 17.8  | 17.8  | 0.035 | 0.023 | 0.003                  | NF 2,000 | 82          |
| 78                                | 0.075                | 1.45 | 0.008 | 0.013 | 2.00 | 0.10 | 17.8  | 17.7  | 0.033 | 0.031 | 0.009                  | NF 2,000 | 84          |
| 74                                | 0.072                | 1.54 | 0.009 | 0.015 | 1.99 | 0.10 | 18.0  | 18.1  | 0.030 | 0.017 | 0.010                  | NF 2,000 | 752         |
| 79                                | 0.081                | 1.45 | 0.014 | 0.013 | 2.00 | 0.10 | 17.8  | 17.8  | 0.034 | 0.036 | 0.009                  | NF 2,000 | 674         |
| Commercial Steels                 |                      |      |       |       |      |      |       |       |       |       |                        |          |             |
| AISI 304L                         | 0.029                | 1.28 | 0.019 | 0.015 | 0.35 | ND   | 9.52  | 18.6  | 0.19  | 0.040 | 0.02                   | 5        | 2           |
| AISI 316                          | 0.061                | 1.69 | 0.027 | 0.029 | 0.35 | ND   | 12.06 | 18.09 | 2.31  | 0.041 | ND                     | 8        | 4           |
| AISI 310                          | 0.063                | 1.15 | 0.024 | 0.013 | 0.32 | ND   | 20.0  | 24.5  | 0.15  | 0.038 | 0.01                   | 15       | 11          |
| Incoilo 800                       | 0.038                | 0.83 | 0.017 | 0.005 | 0.33 | 0.31 | 32.1  | 20.2  | 0.074 | 0.013 | 0.24                   | 1,189    | 167         |

NOTE.—NF=No failure at indicated times; E=Erratic behavior; ND=Not determined.

As is seen from the above, the invention involves an austenitic stainless steel with good corrosion properties, resistance to stress-corrosion cracking in hot chloride environments, and good hot workability. These properties are achieved by a carefully balanced composition which is especially critical because of the interacting effects of carbon and nitrogen, phosphorus and nickel, and phosphorus and silicon. A range of optimum compositions is achieved within the scope of our invention by the effect of crack-retarding elements (nickel, carbon and silicon) overcoming the effect of crack-promoting elements (molybdenum, phosphorus, nitrogen, chromium and sulfur). Furthermore, the effects of austenitizing elements (carbon, manganese, nickel and nitrogen) as provided herein are greater than that of the ferritizing elements (chromium, molybdenum and silicon) so as to produce an austenitic structure.

However, as discussed above, there are additional and other surprising advantages of steels in accordance with the invention. Unlike some generally similar but actually different compositions, our steel possesses a high degree of resistance to high-temperature oxidation as well as to pitting and acid corrosion. The following examples demonstrate these outstanding properties in addition to the stress-corrosion resistance discussed above.

TABLE X  
Resistance to pitting corrosion in a ferric chloride solution

| Alloy:   | Corrosion rate, m.d.d. <sup>1</sup> |
|----------|-------------------------------------|
| 78       | 310                                 |
| 84       | 550                                 |
| Type 304 | 390                                 |

30 <sup>1</sup> M.d.d.—Milligrams per square decimeter per day.

Resistance to acid corrosion is evaluated by testing in a deaerated 10% sulfuric acid at 86° F. for 96 hours. The corrosion rates calculated as mils per year (m.p.y.), a unit commonly used within the chemical industry to describe general or uniform corrosion, are an indication of the steels' acid-corrosion resistance. The results of the acid-corrosion tests are described in Table XI which shows that the corrosion rates of Alloy 78 and Alloy 84 were about an order of magnitude lower than Type 304 stainless, and therefore, superior to it in this property. It is further noted, however, that the corrosion rate of Alloy 78 was appreciably lower than that of Alloy 84.

TABLE XI  
Resistance to corrosion in 10% sulfuric acid

| Alloy:   | Corrosion rate, m.p.y. <sup>1</sup> |
|----------|-------------------------------------|
| 78       | 2.1                                 |
| 84       | 3.7                                 |
| Type 304 | 22                                  |

70 <sup>1</sup> M.p.y.—Mils (0.001 in.<sup>2</sup>h) per year.

The properties of steel in accordance with the invention with respect to high-temperature oxidation resistance also materially contributed to broader application. In a series of tests in which Alloy 78, Alloy 84 and Type 310

stainless steel were tested for high-temperature oxidation resistance, the steel in accordance with the invention demonstrated a degree of resistance comparable to Type 310 stainless which is a material frequently recommended for such applications. The test was performed at temperatures of 1800 and 2000° F. for a period of 8 days. Because oxidation rate varies with time, the test results are expressed as weight loss in milligrams per square decimeter in the 8 days of tests. The results are summarized in Table XII and show that at both temperatures Alloy 78 has had an oxidation resistance essentially the same as Type 310 stainless and both Alloy 78 and Type 310 stainless performed appreciably better than Alloy 84 in this test.

TABLE XII.—RESISTANCE TO HIGH-TEMPERATURE OXIDATION

| Alloy    | Weight Loss in 8 days, mg./dm. <sup>2</sup> |           |
|----------|---------------------------------------------|-----------|
|          | 1,800° F.                                   | 2,000° F. |
| 78       | 290                                         | 690       |
| 84       | 420                                         | 1,180     |
| Type 310 | 280                                         | 780       |

It is apparent from the above that the balanced steel composition in accordance with the invention provides superior properties with respect to a number of important corrosion environments. It is unusual for a single steel to possess a combination of properties as described above in connection with steels in accordance with the invention. While some steels have been provided with stress-corrosion resistance, the steel composition in accordance with the invention is the only one known to possess the variety of outstanding properties as described herein. This outstanding combination of properties is achieved by carefully balancing the composition. However, other elements may be incorporated within the steel to perform known

functions. Thus, for example, where it is desirable to avoid carbide precipitation as a continuous grain boundary network, elements such as titanium, columbium, zirconium and tungsten may be added to minimize or avoid this problem. These elements can be added in amounts which will tie up carbon and/or nitrogen with the net result of minimizing or precluding a decrease in stress-corrosion resistance while alleviating the continuous grain boundary network problem.

We claim:

1. A balanced austenitic stainless steel having good hot workability, stress-corrosion resistance, pitting and acid-corrosion resistance, as well as high-temperature oxidation resistance, consisting essentially of 0.05 to 0.15% carbon, 1.0 to 2.5% manganese, 0.02% max. phosphorus, 0.03% max. sulfur, 1.65 to 3.0% silicon, 15.0 to 19.0% nickel, 15.0 to 19.0% chromium, 0.05% max. nitrogen and 0.05% max. molybdenum.

2. A balanced austenitic stainless steel in accordance with claim 1 having 0.06 to 0.09% carbon, 1.0 to 2.0% manganese, 0.01% max. phosphorus, 0.01% max. sulfur, 1.8 to 2.2% silicon, 15.0 to 19.0% nickel, 17.0 to 19.0% chromium, 0.05% max. nitrogen and 0.02% max. molybdenum.

#### References Cited

##### UNITED STATES PATENTS

|           |         |                      |
|-----------|---------|----------------------|
| 1,745,360 | 2/1930  | Antoinette.          |
| 2,590,835 | 4/1952  | Kirkby.              |
| 2,820,708 | 1/1958  | Waxweiler.           |
| 3,152,934 | 10/1964 | Lula _____ 75—128    |
| 3,276,864 | 10/1966 | Loginow _____ 75—128 |

HYLAND BIZOT, Primary Examiner

UNITED STATES PATENT OFFICE  
CERTIFICATE OF CORRECTION

Patent No. 3,523,788

August 11, 1970

John F. Bates et al.

It is certified that error appears in the above identified patent and that said Letters Patent are hereby corrected as shown below:

Column 8, line 36, "closely" should read -- clearly --; line 41, "various" should read -- various --. Columns 9 and 10, Table VII, line 20, under the heading "Cold Worked" "29" should read -- 2 --; line 21, under the heading "Cold Worked" "72" should read -- 2 --. Columns 11 and 12, Table VIII, line 6, under the heading "Cold Worked", "E 1,64" should read -- E 1,649 --; line 8, under the heading "Cold Worked", "1,013" should read -- 1,012 --; line 9, under the heading "Cold Worked", "82" should read -- 823 --. Table IX, line 1, under "N", "0.038" should read -- 0.031 --; line 2, under "N", "0.021" should read -- 0.029 --; line 3, under "N", "0.039" should read -- 0.036 --; line 4, under "N", "0.026" should read -- 0.028 --. Column 12, lines 54 and 55, "described" should read -- describe --. Column 13, line 11, "essentiatlly" should read -- essentially --.

Signed and sealed this 23rd day of March 1971.

(SEAL)

Attest:

EDWARD M. FLETCHER, JR.  
Attesting Officer

WILLIAM E. SCHUYLER, JR.  
Commissioner of Patents